

## UNITED STATES PATENT OFFICE.

GEORGE C. HALE AND FREDRICH OLSEN, OF DOVER, NEW JERSEY.

## PROPELLENT POWDER.

No Drawing.

Application filed November 6, 1923. Serial No. 673,126.

(GRANTED UNDER THE ACT OF MARCH 3, 1883; 22 STAT. L. 625.)

*To all whom it may concern:*

Be it known that we, GEORGE C. HALE and FREDRICH OLSEN, citizens of the United States, and residents of Dover, in the county of Morris and State of New Jersey, have invented an Improvement in Propellant Powders, of which the following is a specification.

The invention described herein may be used by the Government, or any of its officers or employees in prosecution of work for the Government, or by any other person in the United States, without payment to me of any royalty thereon, in accordance with the act of March 3, 1883.

The subject of this invention is a propellant powder.

The primary object of our invention is the provision of a powder which is nonhygroscopic and which will possess the necessary ballistic qualities.

With the foregoing and other objects in view, our invention resides in the novel combination of ingredients and in the details of preparation hereinafter described and claimed, it being understood that changes in the precise embodiment of the invention herein disclosed may be made within the scope of what is claimed without departing from the spirit of the invention.

Pentaerythritetranitrate and nitroguanidine have many properties which indicate their suitability for use as propellant powders. For example, both are stable compounds, are nonhygroscopic, are easily ignited and burn quietly without leaving any appreciable residue. Heretofore, nitrocellulose has been most generally used as the chief constituent of propellant powders. This material, however, is hygroscopic and powders in which it is used as an ingredient are subject to deterioration due to the effects of dampness and moisture. As it is desirable, therefore, in the development of propellant powders to avoid the use of nitrocellulose because of its hygroscopicity, it is obviously desirable to use such compounds as pentaerythritetranitrate and nitroguanidine, either used alone or mixed with other suitable ingredients which are like pentaerythritetranitrate and nitroguanidine, nonhygroscopic.

It has been found that successful propellant powders may be prepared from pentaerythritetranitrate and nitroguanidine by

mixing these substances with a suitable deterrent material such as triphenylphosphate. Powders containing pentaerythritetranitrate or nitroguanidine and a suitable deterrent will burn with a low flash, producing little smoke and inappreciable residue and will give a uniform velocity.

A composition which has given successful results in practice is as follows:

|                      | Per cent. | 65 |
|----------------------|-----------|----|
| P. E. T. N.          | 21        |    |
| Nitroguanidine       | 41        |    |
| Triphenylphosphate   | 6         |    |
| Ammonium perchlorate | 32        |    |

While it has been found desirable to mix both P. E. T. N. and nitroguanidine with other suitable nonhygroscopic substances, either of these materials may be used alone or combined as a separate ingredient with the proper nonhygroscopic materials. In the formula given above, the proportions of the ingredients used may be varied to suit varying conditions and for the triphenylphosphate any other suitable deterrent such as mononitronaphthaline, dimethylidiphenylurea, dinitrotoluene, etc., may be substituted in the proper proportions, while instead of ammonium perchlorate, any other suitable oxidizing agent may be employed.

A powder made according to the formula given above or employing any other mixture of pentaerythritetranitrate and nitroguanidine or these substances alone with other suitable nonhygroscopic materials may be prepared by any suitable method. The materials either dry or with any desirable moisture content will be mixed together and the mixture pressed into pellets or blocks to a suitable density and these pellets or blocks then granulated to the size desired. Fines which result from such granulation will be returned to the press and repelleted and regranulated until all the powder lies between the limits desired for the granulation. A powder containing ingredients such as recited above and prepared according to the process described will burn very uniformly, largely because of the fact that the repressing of the fine materials assists greatly in the proper incorporation of the various ingredients into the whole mixture. A number of powders have been prepared according to the manner described and with constituents such as recited and have been found to give even

greater uniformity than is obtainable with the standard nitrocellulose powder.

While propellant such as forms the subject of our invention will preferably be prepared according to the method described, it is by no means intended to limit the invention to a powder prepared according to this process alone inasmuch as the materials which we have found desirable to employ may be mixed according to any other suitable method.

We claim:

1. A propellant powder containing pentaerythritetranitrate, nitroguanidine, triphenylphosphate and ammonium perchlorate.
- 15 2. A propellant powder containing pentaerythritetranitrate, nitroguanidine, triphenylphosphate and an oxidizing agent.
3. A propellant powder containing pentaerythritetranitrate, nitroguanidine, a deterrent and ammonium perchlorate.
- 20 4. A propellant powder containing pentaerythritetranitrate, nitroguanidine, a deterrent and an oxidizing agent.
- 25 5. A propellant powder containing pentaerythritetranitrate, nitroguanidine and an oxidizing agent.
- 30 6. A propellant powder containing pentaerythritetranitrate, nitroguanidine and a deterrent material.

7. A propellant powder containing pentaerythritetranitrate, and nitroguanidine.

8. A propellant powder containing nitroguanidine, triphenyl phosphate and ammonium perchlorate.

35 9. A propellant powder containing nitroguanidine, triphenyl phosphate and an oxidizing agent.

10. A propellant powder containing nitroguanidine, a deterrent, and an oxidizing agent.

11. A propellant powder containing nitroguanidine and ammonium perchlorate.

12. A propellant powder containing nitroguanidine and triphenylphosphate.

45 13. A propellant powder containing pentaerythritetranitrate, triphenylphosphate and ammonium perchlorate.

14. A propellant powder containing pentaerythritetranitrate, a deterrent and an oxidizing agent.

15. A propellant powder containing pentaerythritetranitrate, and ammonium perchlorate.

50 16. A propellant powder containing pentaerythritetranitrate, and triphenylphosphate.

GEORGE C. HALE.  
FREDRICH OLSEN.